

## UNITED STATES PATENT OFFICE.

FRITZ SOMMER, OF BERLIN-CHARLOTTENBURG, AND MAX GROTH, OF BERLIN-ORANIENBURG, GERMANY, ASSIGNORS TO THE FIRM CHEMISCHE WERKE VORMALS AUERGESELLSCHAFT M. B. H. KOMMANDITGESELLSCHAFT, OF BERLIN, GERMANY, A CORPORATION OF GERMANY.

## PROCESS FOR PRODUCING ENAMELS AND GLAZES.

No Drawing.

Application filed May 17, 1923. Serial No. 639,714.

*To all whom it may concern:*

Be it known that we, FRITZ SOMMER and MAX GROTH, both citizens of the German Empire, residing at Berlin-Charlottenburg,

5 Germany, and Berlin-Oranienburg, Germany, respectively, have invented certain new and useful Improvements in Processes for Producing Enamels and Glazes, of which the following is a specification.

10 This invention has reference to the elimination of the so-called blistering or bubbling phenomenon occurring in the heating of various enameling or glazing compositions and it is intended to devise means of 15 producing a glaze or enamel which is free from that objectionable quality and to generally improve and perfect the manufacture of compositions of the kind referred to. The utilization of a great number of other- 20 wise very satisfactory opacifiers for glazes or enamels or the like is greatly interfered with by the said phenomenon which the compositions referred to produce upon subsequent firing. Various attempts to 25 overcome this drawback heretofore made have not been successful.

In accordance with this invention, however, it has been ascertained that certain substances, such as burnt clay and similar 30 substances if added to the opacifiers in the grinding mill will increase the opacity and will prevent the very noxious inconvenience of blistering or bubbling of the composition, if these additions before being em- 35 ployed are submitted to a moderately high firing temperature below 1000 degrees centi-grade. The favorable action of such ad- 40 ditions becomes particularly noticeable when using zirconium-oxide for the purpose of producing the opacity but the invention is by no means restricted thereto.

In carrying out the process of this invention the burnt clay or kaolin with the other ingredients, such as unburnt clay, 45 kaolin, and the like are preferably added to the glazing or enameling composition in the grinding mill for instance. It is ob- 50 vious, however, that this invention is not restricted to any particular form of execu- 55 tion and embodiment, but it is susceptible of various changes and modifications to suit,

existing conditions without deviating from the spirit of the invention, as pointed out in the claims, and it should be understood that it is not confined to any particular 55 opacity producing oxide or compound, and that instead of clay any suitable argillaceous or clay containing ingredients may be used.

It is customary in preparing enamels to grind them with clay, and not over 12 per- 60 cent, but usually with 6 to 8 percent unburnt clay. It is this clay that we substitute partially by moderately burnt clay, and the quantity of burnt clay substituted cannot be fixed, as this will vary according to the 65 heat, the composition of the enamel and the effect to be produced, but it may amount to more or less than half the unburnt clay. The quantity to be used will readily be ascertained by the user of the enamels for the 70 conditions existing in the plant.

We claim:

1. The process of improving enameling and glazing compositions, which comprises incorporating both unburnt clay and burnt 75 clay in the enamel.

2. The process of improving enameling compounds containing unburnt clay, which comprises grinding with said compounds a quantity of moderately burnt clay. 80

3. The process of improving enamels or glazes containing zirconium compounds and un-burnt clay, which comprises incorporating with the compounds in the enamel or glaze a quantity of moderately burnt 85 argillaceous material.

4. The process of improving enamels or glazes which comprises burning an argilla- 90 ceous compound at a temperature below 1000° C., and grinding therewith a zirconium compound, a flux and unburnt clay.

5. An enameling or glazing composition containing unburnt and moderately burnt clay.

6. An enameling and glazing compound 95 containing an opacity compound, a flux, unburnt clay and moderately burnt clay.

In testimony whereof we affix our signatures.

DR. FRITZ SOMMER.  
MAX GROTH.